

## UNITED STATES PATENT OFFICE

2,428,404

## ELECTRODEPOSITION OF MOLYBDENUM-COBALT ALLOYS

Leonard F. Yntema, Waukegan, Ill., assignor to  
President & Board of Trustees of St. Louis  
University, St. Louis, Mo.

No Drawing. Application April 24, 1944,  
Serial No. 532,526

5 Claims. (Cl. 204—43)

1

The invention relates to the electrocodeposition of an alloy of molybdenum and a metal of the class consisting of cobalt and iron from aqueous solutions.

I have discovered that such alloys may be codeposited from aqueous solutions when the molybdenum is present in the solution in the hexavalent form, when free alkali metal hydroxide is present and when there is an addition agent capable of holding the cobalt or iron in solution.

In preparing the electrolyte, the molybdenum is added to the water in the form of the alkali metal salt, or, if desired, it may be added as molybdic acid or its anhydride, in which case it is converted into the molybdate form by the free alkali hydroxide. It is essential that free alkali hydroxide be present in the electrolyte during the electrodeposition and it is preferable that the electrolyte also contain alkali metal carbonate. The cobalt or iron is added in the form of a salt such as sulfate, chloride, etc., but to maintain the same in solution it is necessary to add an organic compound having a hydroxyl group and capable of forming complexes with the cobalt or iron. Examples of such organic compounds are sugars, glycerine, glycols and tartaric acid. Inorganic compounds such as phosphates, sulfates and cyanides will not function for this purpose. Preferably I use dextrose.

The electrolyte must be strongly alkaline and good deposits are obtained from a solution containing 250 grams per liter of sodium hydroxide and 80 grams per liter of sodium carbonate. The current density may be varied from 0.03 ampere per square decimeter to 0.5 or higher. Deposits may be obtained at room temperatures or at higher temperatures. I have obtained satisfactory deposits on cathodes of copper and iron. The molybdenum-cobalt plates are bright, very hard and adherent, and are resistant to tarnishing by the atmosphere and to the action of a 3% sodium chloride solution.

I have been unable to obtain alloys of molybdenum with nickel, zinc, tin or bismuth. While I do not wish to be limited to any particular theory as to the operation of my process, it is my understanding that cobalt and iron function as they do because their hydroxides are slightly soluble in strong alkalies. It is possible that the hydrogen, which is discharged as atomic hydrogen along with the cobalt or iron and is dissolved in or is absorbed by them, reduces the molybdenum compounds to the metal by a secondary reaction. This picture of the mechanism of the reaction is based on the facts that no molybdenum is

2

deposited as metal unless cobalt or iron is present, that nickel does not function because its hydroxide is not soluble in the alkaline solutions, and that iron functions better when in the ferric state, which should be more soluble in the strong alkali than the ferrous form. It is my understanding that atomic hydrogen does not dissolve as readily in zinc, tin, and bismuth and therefore these metals do not function.

10 The following is an example of a suitable electrolyte for codeposition of an alloy of molybdenum and cobalt in accordance with my invention:

|    |                  | Range  | Optimum |
|----|------------------|--------|---------|
| 15 | Water            | liters | 1       |
| 20 | Sodium molybdate | grams  | 20      |
|    | Cobalt sulfate   | do     | 10      |
|    | Sodium hydroxide | do     | 250     |
|    | Sodium carbonate | do     | 80      |
|    | Dextrose         | do     | 20      |

What I claim as my invention is:

1. The process for electrodepositing an alloy of molybdenum and a metal of the class consisting of cobalt and iron which consists in passing a current between an anode and the work to be plated as a cathode in an aqueous electrolyte consisting essentially of 10 to 30 grams per liter of

30 a hexavalent molybdate compound, 5 to 15 grams per liter of a soluble compound of a metal of the class consisting of cobalt and iron, 100 to 300 grams per liter of free alkali metal hydroxide and 10 to 30 grams per liter of an organic compound 35 having a hydroxyl group of the class consisting of sugars, glycerine, glycols and tartaric acid.

2. The process for electrocodepositing an alloy of molybdenum and cobalt which consists in passing a current between an anode and the work

40 to be plated as a cathode in an aqueous electrolyte consisting essentially of 10 to 30 grams per liter of a hexavalent molybdate compound, 5 to 15 grams per liter of a soluble cobalt compound, 100 to 300 grams per liter of free alkali metal hy-

45 droxide, and 10 to 30 grams per liter of an organic compound having a hydroxyl group of the class consisting of sugars, glycerine, glycols and tartaric acid.

3. The process for electrocodepositing an alloy 50 of molybdenum and cobalt which consists in passing a current between an anode and the work to be plated as a cathode in an aqueous electrolyte consisting essentially of alkali metal molybdate from 10 to 30 grams per liter, cobalt sulfate 5 to 15 grams per liter, alkali metal hy-

droxide 100 to 300 grams per liter, alkali metal carbonate 40 to 120 grams per liter and an organic compound having a hydroxyl group of the class consisting of sugars, glycerine, glycols and tartaric acid 10 to 30 grams per liter.

4. An electrolyte for the codeposition of an alloy of cobalt and molybdenum consisting essentially of

|                  |        |          |
|------------------|--------|----------|
| Water            | liters | 1        |
| Sodium molybdate | grams  | 20       |
| Cobalt sulfate   | do     | 10       |
| Sodium hydroxide | do     | 250      |
| Sodium carbonate | do     | 80       |
| Dextrose         | do     | 10 to 30 |

5. The process for electrocodepositing an alloy of molybdenum and cobalt which consists in passing a current between an anode and the work to be plated as a cathode in an aqueous electrolyte consisting essentially of alkali metal molybdate

from 10 to 30 grams per liter, cobalt sulfate 5 to 15 grams per liter, alkali metal hydroxide 100 to 300 grams per liter, alkali metal carbonate 40 to 120 grams per liter, and dextrose 10 to 30 grams per liter.

LEONARD F. YNTEMA.

#### REFERENCES CITED

The following references are of record in the 10 file of this patent:

#### UNITED STATES PATENTS

|           |      |              |
|-----------|------|--------------|
| Number    | Name | Date         |
| 1,885,700 | Fink | Nov. 1, 1932 |

#### FOREIGN PATENTS

|         |               |              |
|---------|---------------|--------------|
| Number  | Country       | Date         |
| 1,183   | Great Britain | 1852         |
| 582,528 | Germany       | May 22, 1934 |